

# United States Patent Office

3,078,163

Patented Feb. 19, 1963

1

3.078.163

## SPOT PREVENTION IN LIGHT-SENSITIVE SILVER HALIDE EMULSION LAYERS

Jozef Frans Willems and Gerard Michiel Sevens, Wilrijk-Antwerp, Belgium, assignors to Gevaert Photo-Produchten N.V., Mortsel-Antwerp, Belgium, a Belgian company

No Drawing. Filed Nov. 29, 1960, Ser. No. 72,300  
Claims priority, application Belgium Dec. 2, 1959

4 Claims. (Cl. 96—67)

This invention relates to a method for preventing the formation of small spots caused by the presence of heavy metals and/or their compounds in photographic silver halide emulsions.

During casting and further processing of photographic material, great difficulties sometimes arise the causes of which are not always known. One of the main difficulties is the dust which during the whole cycle of the preparation can set down onto the photographic element.

Since drying the cast photographic layers requires quite a lot of air and since without special precautions this air is polluted by dust particles, it is evident that much dust sets down onto the still moist and sticky coated photographic layer. This evil can practically completely be remedied by thoroughly filtrating the drying air so that practically all dust particles are removed. The drying air, however, is not the only cause of dust. Also the coating machines, the transport machines and the whole manufacturing machinery, the buildings, the persons involved in the manufacture and their clothes can give rise to the formation of dust particles. On considering also the dust caused by corrosion of the coating material, then it will easily be understood that it is quite a problem to manufacture a photographic material in a completely dust-free atmosphere.

As a matter of fact, even if precautions are taken in all manufacturing steps in order to reduce dust formation to an absolute minimum, this does not prevent the settling of minimal traces of dust onto the manufactured material.

The dust itself has a very complex composition. The most occurring elements are vegetable and animal fibres such as paper dust and textile fibres, further soot, sand, insects, rust and fine metal particles. Some of these elements do not cause a chemical reaction on the photographic emulsion and the particles which notwithstanding the extremely careful precautions might set down onto the light-sensitive silver halide emulsion, are so small and in so limited a number that they do not cause any visible faults in the finished photographic material.

More harm is done, however, by the chemically active substance which by its secondary reaction with the emulsion enlarges the caused faults, not visible to the naked eye, and which according to the nature of the dust and the emulsion occasions during processing the exposed material the appearance of small light and dark spots. Chemically reactive dust is mainly composed of metal particles or metal compounds among others metal oxides, especially of heavy metals such as iron, copper, tin, lead, chromium and nickel. These metal particles or metal compounds mainly originate from the construction material of the coating machinery and the working up machines.

Sometimes, however, the used photochemicals contain traces of these metals or of metal compounds, whilst they can also further be present in the used supports such as paper, film and glass on which the light-sensitive emulsions are coated.

The metal particles can be affected more or less slowly in the photographic layers and the formed corrosion products can diffuse away from the central nucleus. These corrosion products can exert either a sensitizing or a de-

2

sensitizing action on the emulsion so that after normal bath treatment of the photographic element a black spot or a white spot respectively, is formed.

Further, most of these metals or their compounds can have a reducing effect and cause a spontaneous development which leads to small black spots. Other influences such as affection of the latent image and hindrance of development lead in their turn to small white spots. In all these cases, the formed small spot is always much larger than the dust particle which is the cause of this undesirable phenomenon. This can easily be checked for instance by bleaching out the silver with a usual oxidation means in the material showing a black spot. The black spots mostly disappear but in the central part remains a very small nucleus which is only visible on enlargement.

Also fine metal particles or dust particles consisting of metal compounds which are present in a non-light-sensitive but adjacent layer, exerts a practically same disadvantageous effect on the superposed or subjacent light-sensitive layer. The harmful corrosion products of the metal particles or the dissolved elements of the metal compounds can indeed reach into the light-sensitive layer by diffusion and cause therein the above mentioned faults.

Now we have found that the formation of spots in photographic images can be avoided by adding to one or more layers which are used for the composition of the photographic material, compounds according to one of the general formulae



· and



40 wherein

$R_1$  and  $R_2$  each represents a member selected from the group consisting of a hydrogen atom, an alkyl group, an hydroxyalkyl group, a formyl group, a carboxyl group, a carbalkoxy group, a phenyl group and a furyl group;  
 45  $R_3$  represents a member selected from the group consisting of a hydrogen atom and an acyl group;  
 $R_4$  represents a member selected from the group consisting of a hydrogen atom, a phenyl group and a p-carboxy phenyl group, and  
 50  $R_5$  represents a member selected from the group consisting of a hydrogen atom and an alkyl group.

Hereinafter follow some examples of suitable compounds:



$\alpha$ -Acetoxyacetyl acetic acid ethyl ester  
 $\text{HOOC-COOH-COOH}$   
Dihydroxymaleic acid  
 $\text{H}_3\text{C-CO-CHOH-CH}_3$   
3-hydroxy-2-butanone (or acetoin)  
 $\text{H}_3\text{C-CO-CHOH-CH}_3$   
5-hydroxy-4-octanone (or butyroin)

3



The compounds according to the present invention can be added in different amounts to the emulsions according to the compounds chosen, the nature of the colloid binding agent for the silver halide grains and the amount and the nature of the silver halide used. Amounts of 0.5 to 2.5 g. per 10 g. of silver metal present in the emulsion as silver halide are preferably used although larger amounts may be added in case it might become necessary. They can, moreover, successfully be added to other layers than the light-sensitive layers such as for instance to a protective layer, an intermediate layer or a baryta-coating.

Evidently, the method according to the present invention can be applied for the manufacture of photographic light-sensitive film as well as of photographic paper.

The use of these compounds for counteracting the formation of spots in photographic images has the advantage of not being accompanied by any harmful secondary effect. On the contrary, some of these compounds when added to a silver chloro-bromide emulsion, increase to some extent the general light-sensitivity of this emulsion without noxious influence on the photographic properties pursued, such as for instance fog and stability.

A further advantage is that the compounds according to the present invention are well compatible with the other emulsion additives such as for instance dispersing agents, color couplers, surface-active compounds, optical bleaching agents, anti-oxidizing agents, sensitizers, anti-fogging agents, stabilizers, hardeners or plasticizers, etc.

The present invention is illustrated by the following examples without limiting, however, the scope thereof.

#### Example 1

Part of a flowable silver chloro-bromide emulsion with pH 4.5 (about 20% of silver bromide) for being applied to paper base is coated onto a strip of baryta-coated paper soiled with metal dust (test strip A); to another part of this emulsion 20 cm.<sup>3</sup> of a 5% alcoholic solution of alpha-acetoxy-acetyl acetic acid ester are added per kg. of emulsion and this second part of emulsion is coated onto a second strip of the same baryta-coated paper (test strip 75

B); to a third part of this emulsion 20 cm.<sup>3</sup> of a 5% alcoholic solution of triosereductone are added per kg. of emulsion whereafter also this third emulsion part is coated onto a third strip of the same baryta-coated paper (test strip C).

These three test strips are dried and exposed in such a way that after development a density of 0.6 is attained. After development, it appears that test strip A shows numerous small black spots having a density which is considerably higher than 0.6. This is not the case for the test strips B and C. Moreover, an increase of sensitivity of 20% has been observed on test strip C, without further influence on the gradation and other photographic characteristics.

#### Example 2

Part of a warm-tone silver chloro-bromide emulsion with pH 4.7 (about 30% of silver bromide) for being applied onto paper base is coated onto a strip of baryta-coated paper soiled with metal dust (test strip A); part of this material is provided with an antistress layer mainly composed of gelatin. To the usual coating composition from which this antistress layer is coated 25 cm.<sup>3</sup> of a 5% alcoholic solution of 3-methyl-4,5-dihydroxypyrazole were added per litre (test strip B); another part of this paper is likewise coated with the same antistress layer not containing however 3-methyl-4,5-dihydroxypyrazole (test strip C). After exposure and development to low density, the test strip B does not show black spots, whereas the test strips A and C show many small black spots.

#### Example 3

A strip of a paper support with metal dust is provided with a gelatin precoat containing an antihalation substance (test strip A); to a second strip of the same paper support likewise soiled with metal dust a gelatin precoat is applied from a coating solution which, however, besides the same antihalation substance as in strip A, 40 cm.<sup>3</sup> of a 5% alcoholic solution of 1-phenyl-3-methyl-4,5-dihydroxypyrazole were added per 1 litre of coating solution (test strip B); to a third strip of the same paper support a gelatin precoat is applied from a coating solution to which, however, besides the same antihalation substance as in strip A, 20 cm.<sup>3</sup> of a 5% alcoholic solution of 1-p-carboxyphenyl-3-methyl-4,5-dihydroxypyrazole per litre of coating solution were added.

On the precoat of each test strip is coated the same silver-chloride emulsion with pH 5, suitable for the preparation of aluminum offset sheets such as described in the U.S. patent application Serial No. 846,256, filed October 14, 1959.

Contrary to test strip A, the test strips B and C after exposure and development show a homogeneous density without black spots.

We claim:

1. A photographic material comprising a support and at least one layer superposed thereon, one such layer being a light-sensitive silver halide emulsion layer, said material being characterized in that at least one of the layers thereof contains a compound having a formula selected from the group consisting of:



and



70 wherein

$\text{R}_1$  and  $\text{R}_2$  each represents a member selected from the group consisting of a hydrogen atom, a methyl group, an ethyl group, a propyl group, an hydroxymethyl group, a formyl group, a carboxyl group, a

carbethoxy group, a phenyl group and a furyl group; R<sub>3</sub> represents a member selected from the group consisting of a hydrogen atom and an acetyl group, and R<sub>4</sub> represents a member selected from the group consisting of a hydrogen atom, a phenyl group and a p-carboxy phenyl group, whereby the formation in said emulsion layer spots caused by dust such as metallic particles and the like is substantially inhibited.

2. A photographic material having a light-sensitive 10 silver halide emulsion layer containing alpha-acetoxy-acetyl acetic acid ethyl ester.

3. A photographic material having a light-sensitive silver halide emulsion layer and an antistress layer containing 3-methyl-4,5-dihydroxypyrazole.

4. A photographic material having a light-sensitive silver halide emulsion layer and a gelatin precoat containing 1 - (p-carboxyphenyl)-3-methyl-4,5-dihydroxypyrazole.

References Cited in the file of this patent

UNITED STATES PATENTS

2,346,095 Weissberger et al. ----- Apr. 4, 1944